

June 30, 1936.

F. W. ADAMS ET AL

2,045,818

METHOD OF AND APPARATUS FOR PRODUCING PAPER PULP

Filed June 26, 1934

2 Sheets-Sheet 1



*Fig. 1*



*Fig. 2*

INVENTORS:  
Frederick W. Adams  
George S. Whitney  
BY *J. M. Cadey*,  
Their ATTORNEY.

June 30, 1936.

F. W. ADAMS ET AL

2,045,818

METHOD OF AND APPARATUS FOR PRODUCING PAPER PULP

Filed June 26, 1934

2 Sheets-Sheet 2



INVENTORS:  
Frederick W. Adams  
George S. Whitney  
BY  
J. H. McCauley,  
Their ATTORNEY.

## UNITED STATES PATENT OFFICE

2,045,818

METHOD OF AND APPARATUS FOR  
PRODUCING PAPER PULPFrederick W. Adams, Stoneham, Mass., and  
George S. Witham, Jr., Lincoln, N. H.

Application June 26, 1934, Serial No. 732,456

8 Claims. (Cl. 92—7)

This invention relates to the production of chemical wood pulp. It has for its general objects to improve the quality of the pulp obtained from a given grade of wood, and to effect economies in the pulp producing process.

As is well understood by those skilled in this art, the commercial methods of producing pulp of this character include the cooking of wood chips in a large digester. At the completion 10 of the cook, the pulp and digester liquor are discharged into a pit or vat, the discharging operation being commonly referred to as "blowing" the digester, and the pit or vat usually being called a "blow pit." When the charge is 15 ready to be blown, it is under considerable pressure, say for example, between 40 and 120 lbs. per square inch, and its temperature is high, ranging from, perhaps, 270° to 350° F. The blowing operation consists simply in opening the blow valve and allowing the pressure in the digester 20 to force the entire charge through a pipe line into the blow pit, where the pressure is substantially atmospheric. Consequently, when the pulp is discharged, the pressure on the fibers is released very quickly. This sudden release of pressure produces an effect on the fibers similar to that purposely created in a similar manner in some industries for the purpose of "exploding" the product under treatment. In the case of 25 pulp, however, the result is to weaken the fiber and, consequently, to reduce the strength of the paper ultimately made from the fiber.

In addition to this effect, the practice just described also results in producing large volumes 30 of steam which are discharged into the surrounding atmosphere through the vomit stack leading from the blow pit. Small proportions of sulphurous acid are carried off with the steam and gases so evolved and create a nuisance, due partly 35 to their disagreeable smell and partly, also, to their tendency to attack metal roofings and other exposed metal parts of adjacent buildings.

The present invention is especially concerned 40 with these considerations, and it aims to improve processes of handling the pulp in connection with the cooking operation with a view to avoiding the objections just described and conserving the heat contained in the cooked charge, and which, according to the customary process, is wasted.

50 The nature of the invention will be readily understood from the following description when read in connection with the accompanying drawings, and the novel features will be particularly pointed out in the appended claims.

55 In the drawings,

Figure 1 is a side elevation, partly in section, showing somewhat diagrammatically those features of an apparatus with which this invention is more especially concerned;

Fig. 2 is an end view on a larger scale of the 5 float operated valve illustrated in Fig. 1; and

Fig. 3 is a vertical, sectional view of parts of the apparatus shown in Fig. 1.

The apparatus illustrated in the drawings 10 comprises a digester 2, from the bottom of which the usual pipe line or blow line 3 leads into the blow pit 4. Included in the blow line is the usual blow-off valve 5. So far as these features of this arrangement are concerned, they may be of any 15 usual or convenient form.

According to the present invention, an injector 6 is included in the blow line 3, and the intake leg 7 of this injector leads into a well or reservoir 8 which is kept constantly filled to a substantially predetermined level with cold water or other suitable liquid. In the particular construction shown a pipe 9 conducts water from any suitable source into the bottom of the well 8 through a float operated valve 10 which serves to maintain the desired level automatically, an 20 overflow pipe 12 preferably being provided to conduct away the surplus water in the event that the valve fails, for any reason, to operate properly.

When the cook has been completed and the 30 valve 5 is opened to blow the charge, the kinetic energy of the outgoing mixture of pulp and waste digester liquor flowing through the injector creates a suction in the intake leg 7, serving to cause a flow of water from the well 8 through the leg 7 and into the injector where it becomes mixed with the pulp and digester liquor flowing through the pipe line 3. By selecting an injector of a design and capacity suited to the requirements of the individual digester with which it 35 is to be used, and properly controlling the head through which the cooling water must be raised, the proportion of water mixed with the outgoing charge can be predetermined within limits sufficiently accurate for all practical purposes. The 40 quantity of water so mixed with the discharged stock should be sufficient to prevent the formation of any objectionable quantity of steam during practically the entire blow. When the valve 5 is first opened there is a brief instant during 45 which the discharged stock will not be mixed with water, but this interval of time is only momentary, as will readily be appreciated, and is simply long enough to enable the flow of stock to set up the necessary vacuum required to start 50 55

the flow of water through the injector. Thereafter the stock will be discharged into the blow pit in a hot condition but at a temperature below the boiling point of water. With this arrangement, therefore, the explosion of the fiber, and the consequent weakening action on it, is avoided and the creation of large volumes of steam also are prevented.

The mixing of the water with the discharged stock serves not only to cool the pulp, as above described, but it also initiates the pulp washing operation, the water added to the stock being utilized for this purpose. In addition, it permits the washing of the pulp at a higher temperature than that ordinarily used so that this operation is made more effective, more uniform, and proceeds more rapidly. Thus the heat which has been wasted by former processes is conserved and made to serve a useful purpose.

The foregoing operations are typical of those used in the production of chemical wood pulp by the sulphite process. The invention is equally applicable to the sulphate and soda processes. In the latter, however, the water usually will be replaced with black liquor. Here, the invention produces the additional advantage of assisting in the evaporation of the water constituent of the liquor incidental to the usual recovery process.

Preferably a check valve 14, Fig. 3, is located at the intake port of the injector, or at some point in the intake leg 1, where it will prevent any flow downwardly through this leg.

While we have herein shown and described a procedure embodying this invention which is typical of one process of producing pulp, and an apparatus suitable for use in said process, it will be evident that the invention may be embodied in other forms and practiced in other ways without departing from the spirit or scope thereof.

Having thus described our invention, what we desire to claim as new is:

1. The combination with a pulp digester, a blow-off line leading therefrom and a blow-off valve in said line, of means for mixing a sufficient quantity of a suitable liquid with the charge of stock and waste liquor while the stock is flowing through said line to prevent any substantial explosion of the fiber as the latter is discharged from said line.

2. The combination with a pulp digester, a

blow-off line leading therefrom and a blow-off valve in said line, of means for mixing a sufficient quantity of a suitable liquid with the charge of stock and waste liquor while the stock is flowing through said line to prevent the discharge 5 of any substantial quantity of steam from said line during the blowing of a charge.

3. The combination with a pulp digester, a blow-off line leading therefrom and a blow-off valve in said line, of an injector in said line, and 10 a supply of relatively cool liquid with which the intake leg of said injector is connected.

4. The combination with a pulp digester, a blow-off line leading therefrom and a blow-off valve in said line, of an injector in said line, and 15 means for conducting relatively cool liquid to the intake port of said injector.

5. The combination with a pulp digester, a blow-off line leading therefrom and a blow-off valve in said line, of an injector in said line, a 20 well for holding a supply of relatively cool liquid, an intake pipe leading from the intake port of said injector into said well, and a check valve in said pipe serving to prevent any substantial flow of liquid through the pipe from the injector 25 to the well.

6. That improvement in methods of producing chemical wood pulp, which consists in cooking the pulp, blowing the charge at the end of the cook, and causing the kinetic energy of the charge 30 to mix a cooling liquid with the outgoing charge before the charge is liberated.

7. That improvement in methods of producing chemical wood pulp, which consists in cooking the pulp, blowing the charge at the end of the 35 cook, and causing the kinetic energy of the charge to mix a sufficient proportion of a suitable cooling liquid with the outgoing charge, while said charge is still under pressure, to substantially prevent the discharge of steam at the final 40 delivery.

8. That improvement in methods of producing chemical wood pulp, which consists in cooking the pulp, blowing the charge at the end of the cook, and, during said blowing operation, mix- 45 ing a sufficient proportion of a relatively cool liquid with the stream of pulp being discharged to prevent explosion of the fiber upon its final delivery.

FREDERICK W. ADAMS. 50  
GEORGE S. WITHAM, JR.